

Nov. 10, 1942.

W. R. FORSYTHE

2,301,390

PRIMARY CELL

Filed July 8, 1941



Fig. 1



Fig. 2

INVENTOR.

William L. Forsythe

BY

Griswold & Burdick  
ATTORNEYS

## UNITED STATES PATENT OFFICE

2,301,390

## PRIMARY CELL

William R. Forsythe, Midland, Mich., assignor to  
 The Dow Chemical Company, Midland, Mich.,  
 a corporation of Michigan

Application July 8, 1941, Serial No. 401,435

5 Claims. (Cl. 136—100)

This invention relates to an improved primary cell utilizing metallic magnesium as the anode material.

An object of the invention is to provide a primary cell which is capable of a considerably higher energy output per unit weight than cells now in common use. Another object is to provide a cell which is of unusually simple construction and may be readily fabricated from a very few elements. A further object is to provide a cell which is not subject to gassing and does not deteriorate when standing without delivering current. Other objects will be evident from the description.

The essential elements of the new primary cell are an anode composed of metallic magnesium, a cathode of chemically inert electrically conducting material such as carbon or graphite, and an electrolyte in contact with the electrodes and consisting essentially of an aqueous solution of chromic acid.

The anode may be formed either of pure metallic magnesium or of a magnesium-base alloy containing a major proportion of the metal, all such materials being included with the term "magnesium" as hereinafter employed. However, metallic magnesium of at least 99.5 per cent purity is to be preferred because of its somewhat higher electrode efficiency and its higher hydrogen overvoltage.

The electrolyte preferably consists of a water solution of chromic acid, and is conveniently prepared by dissolving chromic anhydride ( $\text{Cr}_2\text{O}_3$ ) in distilled water. Concentrations of chromic anhydride of from 11 parts by weight per 100 parts of water up to a saturating amount are preferred. This electrolyte is inert to the magnesium anode except when the cell is delivering current, and even then does not cause the formation of any significant coating on the electrode.

Small proportions of inert solutes may, of course, be present in the electrolyte without departing from the invention. In general, however, a simple water solution of chromic acid is to be preferred, since the addition of certain common inorganic acids or salts to the chromic acid solution causes it either to attack the magnesium anode by direct chemical action or else to form an impervious coating on the magnesium during operation of the cell.

The invention may be further explained with reference to the accompanying drawing, in which:

Fig. 1 is a diagrammatic vertical section of a simple form of the new cell; and

Fig. 2 is a similar section of another form of the cell.

5 The cell illustrated in Fig. 1 is contained in a jar 3 of an insulating substance such as glass or molded synthetic plastic, fitted with a tight cover 4 of like material, and filled with a water solution of chromic acid 5. Depending into the jar through separate holes in the cover so as to contact the electrolyte are a magnesium rod 6 and a carbon rod 7, each rod being provided with a binding post.

The cell of Fig. 2, which is of the "dry cell" type, is contained in a cup 8 formed of metallic magnesium, the cup also serving as the anode of the cell, and being for this purpose provided with a binding post 9. Fitting closely inside the magnesium cup is a liner 10 separating the anode from the cathode portion of the cell, the liner being formed of a chemically inert electrically non-conducting porous material such as blotting paper, cloth fabric, or the like. Inside the liner the cell is filled with a mass of finely-divided carbon 11, with which a carbon rod 12 extending through the sealed insulating cover 13 is in direct electrical contact. The mass of fine carbon is saturated with a water solution of chromic acid as electrolyte.

20 30 The electrolytic reaction in the new cell is not fully understood, but appears to involve an oxidation at the anode of the metallic magnesium, probably with the formation of magnesium chromate, and a reduction at the cathode of the chromic acid, with liberation of tri-valent chromium salts.

35 The cell develops an open circuit potential of about 1.2 volts, while the energy output per unit weight of cell is considerably in excess of that exhibited even by dry cells of the Leclanche type. In contrast to the latter cell, the shelf life of the new cell is almost indefinite, and gassing at the anode does not occur to any significant extent.

40 It is to be understood that the foregoing description is illustrative rather than strictly limitative, and that other embodiments of the new cell are possible within the spirit of the invention and the scope of the following claims.

I claim:

50 1. A primary cell comprising a magnesium anode and an electrolyte consisting of a water solution of chromic acid.

2. A primary cell comprising a magnesium anode, a carbon cathode, and an electrolyte consisting of a water solution of chromic acid.

3. A cell according to claim 2 wherein the metallic magnesium forming the anode is of at least 99.5 per cent purity.

4. A primary cell in which the essential elements consist of a magnesium anode, a carbon cathode, and an electrolyte consisting of the solution prepared by dissolving at least 11 parts by weight of chromic anhydride in 100 parts of water.

5. A primary cell comprising an anode of metallic magnesium, a cathode formed of a carbon rod surrounded by and in direct electrical contact with a mass of finely-divided carbon, a body of chemically inert electrically non-conducting porous material separating the anode from the cathode mass, and an electrolyte consisting of a water solution of chromic acid.

WILLIAM R. FORSYTHE.